

## UNITED STATES PATENT OFFICE.

ZAY JEFFRIES AND ROBERT S. ARCHER, OF CLEVELAND, OHIO, ASSIGNEES TO AMERICAN MAGNESIUM CORPORATION, OF NIAGARA FALLS, NEW YORK, A CORPORATION OF NEW YORK.

## HEAT TREATING MAGNESIUM ALLOYS.

No Drawing.

Application filed October 14, 1921. Serial No. 507,766.

Our invention relates to the treatment of magnesium-base alloys, that is, those in which the principal metal is magnesium. One of the objects of the invention is to improve the physical properties of these alloys, such as the strength or plasticity, by subjecting them to heat treatment. A further object of the invention is to increase the susceptibility of these alloys to mechanical deforming processes and which is incident to these improved properties. Another object of the invention is to prevent burning of the metal during the heat treatment. With these and other objects in view, our invention consists in certain novel features as will be hereinafter described and particularly pointed out in the claims.

As illustrative of our discovery, we take a magnesium-base alloy casting containing from 3 to 15% aluminum and which may contain in addition thereto, small quantities of other metals such as zinc up to 5%, cadmium up to 10%, copper up to 2%, manganese up to 2%. Such alloy may be in the form of a casting and the casting may be any of the well known types, e. g. green sand, dry sand, semi-permanent mold, permanent mold or die casting.

In carrying out our invention, the metal is subjected to heat treatment at a temperature slightly below the melting point of the most fusible constituent of the alloy for an extended period of time, sometimes as long as 70 hours. With the alloys hereinabove specified the most suitable temperature is between 400-440 degrees C. or about 10-50 degrees C. below the fusing point of the magnesium-aluminum eutectic richest in magnesium.

Heat treatment for shorter periods of time improves the properties of the alloy but not to the extent of longer heat treatment.

The effect of this heat treatment may be indicated by the following example. Magnesium castings containing approximately 5 to 7% aluminum, have a tensile strength after casting in green sand of about 22,000 lbs. per sq. in. and an elongation of 1½ to 3%. After heating for 48 hours at a temperature of 420-430 degrees C. we have secured a tensile strength above 30,000 lbs. per sq. in. and an elongation of more than 8% in two inches.

Magnesium-base alloys containing from 3 to 15% aluminum, with or without small ad-

ditions of other elements, are particularly 55 adapted to this heat treatment.

The increase in plasticity of the metal by heat treatment finds particular application in connection with mechanical deforming processes depending upon plasticity, such as extruding, rolling, drawing and forging. At the present time certain of these alloys cannot be commercially worked. When subjected to the above described heat treatment, the working qualities are materially improved, especially when the metal is hot.

We have also discovered that the heating of the magnesium-base alloys for long periods of time at a temperature of 400 degrees C. or above in an air atmosphere may produce spontaneous burning of the metal. This is more noticeable in some types of alloys than in others and frequently the heat treatment is satisfactory when carried out in an air atmosphere. When it is desired, however, to insure against any trouble from this source, we prefer to put the metal in an iron or other suitable container and maintain an inert atmosphere or vacuum in this container while the metal is at heat.

The theory upon which magnesium-base alloys are improved by heat treatment may be explained in part as follows:

In the casting of alloys composed principally of magnesium and containing other alloying metal, soluble, at least within a certain range of composition, in the magnesium metal in the solid state, the saturation quantity of alloying element is not in solution in the magnesium after casting. Taking the 90 magnesium-aluminum alloys, as an example, the equilibrium diagram would indicate that about 11% of aluminum by weight should be soluble in magnesium at the freezing temperature of the eutectic alloy. In a magnesium casting containing as little as 4 or 5% aluminum a considerable quantity of an aluminum-rich constituent, separates out in a complete or partial net work enclosing, or adjacent to, grains of magnesium-rich constituent. We have discovered that the plasticity of the metal particularly suffers because of this structure and the strength is also relatively low.

An equalization of composition can be effected by heating the castings for a relatively long period of time, sometimes requiring up to seventy hours and we have discov-

ered that the physical properties are very much improved by this heat treatment process.

While we refer herein to the application 5 of the process to castings we do not intend to so limit our discovery, as the same heat treatment could be applied to articles after they have been mechanically worked or shaped, especially if the aluminum content is 10 10% or more.

We claim:

1. The process of working a magnesium base alloy containing a metal capable of dissolving in solid magnesium in an amount 15 greater than found in solution in the alloy as cast comprising subjecting the alloy to a heat treatment at a high temperature but below the melting temperature of the most fusible constituent of the alloy to cause increased solution of the other metal in the solid magnesium, thereby increasing the plasticity of the alloy and then mechanically deforming the 20 alloy while hot.

2. The process of working a magnesium base alloy containing a quantity of aluminum capable of dissolving in solid magnesium in an amount greater than is in solution in the alloy as cast, comprising subjecting the alloy to a heat treatment at a high temperature but 25 30 below the melting temperature of the most fusible constituent of the alloy to cause increased solution of the aluminum in the solid magnesium, thereby increasing the plasticity of the alloy and then mechanically deforming the 35 alloy while hot.

3. The process of working magnesium base alloys containing from 3 to 15% aluminum and capable of dissolving in solid magnesium up to about 11% aluminum and in an amount 40 greater than is in solution in the alloy as cast, comprising subjecting the alloy to a

heat treatment at a high temperature, but below the melting temperature of the most fusible constituent of the alloy to cause increased solution of the aluminum in the solid 45 magnesium, thereby increasing the plasticity of the alloy and then mechanically deforming the alloy while hot.

4. The process of working magnesium base alloys containing a quantity of aluminum capable of dissolving in solid magnesium in an amount greater than is in solution in the alloy as cast comprising subjecting the alloy to a heat treatment at 400-440° C. for a period of hours to cause increased solution of the 50 aluminum in the solid magnesium, thereby increasing the plasticity of the alloy and then mechanically deforming the alloy while hot.

5. The process of working magnesium base 55 alloys containing 3 to 15% aluminum and capable of dissolving in solid magnesium up to about 11% aluminum and in an amount greater than is in solution in the alloy as cast, comprising subjecting the alloy to a heat treatment at 400-440° C. for a period of hours to cause increased solution of the aluminum in the solid magnesium, thereby increasing the plasticity of the alloy, and then mechanically deforming the alloy while hot. 60

6. The process of working magnesium base alloys, comprising subjecting the solid metal to heat treatment at a high temperature for a period of hours but below the melting temperature of the most fusible constituent of 65 the alloy to increase the plasticity of the alloy and thereafter mechanically deforming the alloy. 7

In testimony whereof they affix their signatures.

ZAY JEFFRIES.  
ROBERT S. ARCHER.